

## UNITED STATES PATENT OFFICE

2,170,259

PROCESS FOR THE INTRODUCTION OF  
GRAPHITIC CARBON INTO LIGHT METALS  
OR LIGHT METAL ALLOYS

Heinrich Borofski, Frankfort-on-the-Main, Germany, assignor of one-half to the firm Mettmanner Britannia-Warenfabrik W. Seibel, Mettmann, Rhineland, Germany

No Drawing. Application December 30, 1937, Serial No. 182,544. In Germany January 9, 1936

16 Claims. (Cl. 75—135)

This invention relates to a new or improved process for the introduction of graphitic carbon into light metals or light metal alloys. It is already known that an addition of carbon in the form of graphite, is advantageous, particularly in reducing the co-efficient of friction. This so-called graphiting of metals or alloys was previously effected by introducing graphite powder into the melt. When these graphited metals or alloys are in their melted condition, there is a tendency for separation to take place on account of the great difference between the specific weight of the graphite and that of the metal. To prevent this separation, it has already been proposed to weight the graphite to be introduced into the metal in order to make its specific weight equal to or approximately equal to that of the metal. Attempts have been made to bring about the weighting by galvanically coating the graphite particles with a coating of metal of higher specific weight, for instance of copper or nickel, or by incorporating the graphite in a metal or alloy, and by then introducing the galvanically coated graphite particles or the mixture of graphite and metal into the alloy to be graphited. These attempts, however, have had no success, because, on the one hand, it is difficult to provide a metal coating upon graphite, which travels in the galvanic bath from the cathode to the anode, and, on the other hand, the affinity of the coating and weighting metals to the metal to be graphited or to the alloy to be graphited is of considerable importance, and frequently makes the weighting of the graphite inoperative by alloying the weighting metal with the metal to be graphited. Finally, especially with light metals or light metal alloys which are particularly subject to oxidation it is necessary that in the graphiting no moisture of any kind should be brought into the fluid metal, since thereby the formation of oxide and, in certain circumstances, even the formation of carbides, occurs, and this would make the graphited alloys unserviceable, by reason of the great hardness of the oxides and carbides, for the very purposes in which good ability to slide is concerned. On coating the graphite particles with galvanic metal coatings, fluid occlusions cannot, however, be avoided with certainty.

The invention concerns a process for the production of colloid mixtures from light metals or light metal alloys and carbon especially in the form of graphite, in which the disadvantages of the previously known processes are avoided by using, for weighting the graphite, not pure metals or alloys but metal compounds, for instance me-

tallic salts, which are decomposed before or during graphiting, for example by change of temperature or by chemical reaction, whereby the metal is liberated and the individual graphite particles are weighted. The process may, with advantage, be carried out by stirring up with the graphite a metal compound dissolved in water or other fluid, until the graphite particles are completely moistened or penetrated by the solution and freed from the adhering air, and then removing the fluid, for instance by filtering and evaporation, and introducing the residue into the metal to be graphited.

If, for instance, an aluminium alloy is to be graphited, there is used as a weighting medium for the graphite lead acetate  $Pb(C_2H_3O_2)_2 \cdot 3H_2O$ , for instance, which is completely dissolved in any suitable solvent, for instance, water. The graphite is mixed into this solution and is then freed from adhering air by lengthy stirring and kneading and completely moistened and penetrated by the solution. The mixture of dissolved lead acetate and graphite is preferably left standing for some time and is then again stirred or kneaded. The fluid is now evaporated at temperatures of about  $100^{\circ} C.$  and thereby the water of crystallisation of the lead acetate is also removed and the mass obtained introduced into the fluid aluminium alloy. Even at temperatures below  $200^{\circ} C.$  the lead acetate decomposes. Although acetone and carbonic acid escape, the lead and carbon do not vaporise at the temperatures employed and therefore remain in the mixture and weight the graphite. The weighted graphite permeates the alloy to be graphited in the finest distribution and forms a very stable colloidal mixture with the alloy. An aluminium alloy graphited in this manner possesses an extraordinarily low frictional coefficient which equals and even bettered that of the best white bearing metals.

The invention extends, of course, not only to the graphiting of aluminium alloys by weighting the graphite with the aid of lead acetate, lead chloride or any other lead compound, but is also applicable with advantage to the graphiting of other metals and alloys and employing compounds of other metal as the weighting media for the graphite. In the example described above, a lead compound has been selected as weighting medium because lead has only a small affinity for aluminium, copper, nickel and other metals used for metal alloys. Metal compounds can, however, be used with advantage as weighting media, even for those metals or alloys of which

the main components easily combine with lead. It may be presumed that on mixing the graphite with the lead compound, a complete penetration of the graphite occurs, and thus the air or any other gas adhering or tending to adhere to the graphite particles is displaced, so that the buoyancy of the graphite in the melt is decreased, and the weighting medium is in no case completely dissolved out of the graphite particles.

10 The metal compounds to be employed for weighting the graphite can be so chosen that either one only or several components thereof remain in the alloy to be graphited. When lead acetate is used, carbon also remains in addition to lead in the alloy to be graphited. If required, compounds containing carbon may be added alone to the metal or alloy as the weighting medium, for instance lead acetate by itself without an admixture of graphite, in as far as, during 15 the process, a decomposition of the weighting medium occurs or can be readily caused to occur. Finally, instead of solutions of metal compounds, there may also be used as weighting media suitable mixtures of lead or other metals or alloys and graphite, provided that all the materials are reduced to colloid fineness.

What I claim is:

1. Process for graphiting light metals which comprises mixing graphitic carbon with a decomposable metal compound, introducing such mixture into a melt of said light metal and bringing about decomposition of said metal compound with liberation of metal in close association with said carbon.
2. Process for graphiting light metals which comprises mixing graphitic carbon with a carbon-containing heavy metal compound decomposable to metal and carbon at the melting point of said light metal, and incorporating the mixture in a melt of said light metal.
3. Process for graphiting light metals which comprises introducing into a melt of said light metal a carbon-containing metal compound adapted at the temperature of the melt to be decomposed into metal and carbon and bringing about solidification of the light metal without segregation of such carbon.
4. Process for graphiting light metal which comprises introducing into a melt of said light metal a mixture of graphitic carbon and a metallic salt selected from the group of metallic salts which under the influence of heat liberate metal adapted to associate with graphite particles, and bringing about solidification of the light metal without substantial segregation of carbon.
5. Process as claimed in claim 2 in which the heavy metal compound is an acetate.
6. Process for graphiting light metals which comprises moistening and impregnating graphitic carbon with a solution of a lead salt, expelling air and solvent, incorporating the graphitic carbon so treated in a melt of light metal and solid-

ifying said light metal without segregation of carbon.

7. In a process of incorporating graphitic carbon into light metal the steps which consist in mixing said carbon with a decomposable heavy 5 metal compound containing carbon, and bringing about decomposition of said heavy metal compound with liberation of metal and carbon.

8. Process for graphiting light metal which comprises introducing into a melt of said light 10 metal graphitic carbon and a metallic salt selected from the group of metallic salts which under the influence of chemical substances liberate metal adapted to associate with graphite particles, and bringing about solidification of the 15 light metal without substantial segregation of carbon.

9. The process for graphiting light metals or alloys thereof, which consists in producing a mixture of graphitic carbon with a metal compound 20 which decomposes at the melting temperature of the light metal or alloy to be graphited, introducing said mixture into the molten light metal or alloy, and bringing about solidification of such metal or alloy.

10. Process as claimed in claim 9, in which the mixture of graphitic carbon and decomposable metal compound is in a dry condition at the time of its addition to the molten light metal or alloy.

11. Process as claimed in claim 9, in which a compound of a heavy metal is used as the decomposable metal compound.

12. Process as claimed in claim 9, in which a lead compound is used as the decomposable 35 metal compound.

13. Process according to claim 1, in which a lead compound is used as the decomposable metal compound.

14. Process according to claim 1, in which 40 lead acetate is used as the decomposable metal compound.

15. The process for graphiting light metals or alloys thereof, which consists in mixing graphitic carbon with a solution of a metal compound which decomposes at the melting temperature of the light metal or alloy to be graphited, removing air and the solvent from said mixture of graphitic carbon and metal compound, introducing the resulting dry mixture into the molten 45 light metal or alloy, and bringing about solidification of such metal or alloy.

16. The process for graphiting light metals or alloys thereof, which consists in mixing graphitic carbon with a solution of a decomposable metal compound, removing air and the solvent from said mixture of graphitic carbon and metal compound, introducing the resulting dry mixture into the molten light metal or alloy, and bringing about solidification of such 50 metal or alloy.

HEINRICH BOROFSKI.